

## UNITED STATES PATENT OFFICE

1,982,048

SOLUBLE DRIER FOR PAINTS AND  
VARNISHES

Robert A. Dunham, Long Beach, Calif., assignor  
to Union Oil Company of California, Los An-  
geles, Calif., a corporation of California

No Drawing. Application September 16, 1933,  
Serial No. 689,787

11 Claims. (Cl. 134—57)

This invention relates to driers for paints and varnishes and particularly to the so-called soluble drier class. The object of the invention is to furnish a drier of the stated type which shall have more desirable properties than driers employed heretofore, particularly in that they shall have a higher theoretical manganese value than the average drier heretofore and at least as high as any soluble drier employed in the past, and shall at the same time be more readily miscible and soluble in appropriate agents (e. g. naphtha) than previously known driers.

Driers employed heretofore have usually been prepared from such organic acids as linoleic and abietic ("resinic") acids. These acids are however unsaturated and at the same time possess such a high molecular weight that the theoretical metal content thereof, which is the active constituent, is undesirably low. For instance the theoretical metal content of manganese linoleate is 9.0%. While some other driers have afforded a theoretical manganese content as high as 11%, these have offered the objections that they have been difficult to bring into solution or at least have required very awkward or dangerous procedures.

I have discovered that any one of the common so-called "drying" metals such as cobalt, manganese and the like combine to produce very satisfactory driers with the fatty acids of coconut oil or other equivalent saturated fatty acids, i. e. saturated fatty acids of low molecular weight. These soluble driers possess all the desired properties of ready solubility (as in naphtha) at normal temperatures and have also the desired high metal content. For example the theoretical manganese content of the manganese-coconut acid compound hereof is about 11.5%.

According to the invention the soluble driers hereof may be made by combining with the fatty acids of coconut oil any suitable "drying" metal such as cobalt, copper, lead, manganese and zinc. Oxides or carbonates of these metals preferably are used. The fatty acids of the coconut oil are chiefly capric, lauric and myristic acids. These acids are saturated and are thereby distinguished from the unsaturated linoleic, abietic and other acids heretofore employed. The resultant mixed metal salts of these mixed coconut oil-acids, when in finished form so as to be free of water and oil, possess a waxy consistency and are therefore easy to handle. The manganese-coconut oil drier for example, when stirred in cold naphtha readily forms a fine suspension which is easily converted into a clear solution by heating

to the boiling point of water. The resultant solution does not reprecipitate for several hours after cooling and consequently may be added readily as a liquid drier to any of the paints and varnishes in the small amount required for these purposes. The resultant solution is stable. The products from the type of saturated fatty acids mentioned are less subject to spontaneous combustion and discoloring than the linoleates and resinate and contain no ingredients which are any more deleterious to paints and varnishes than the other soluble driers at present in use. The characteristics above indicated for the manganese-coconut acid drier apply equally well to the characteristics of the driers produced with the other metals mentioned, all these driers having substantially the same desirable characteristics and high content of the active (metal) constituent.

As applied to a manganese-coconut acid drier, one desirable method of manufacture follows, the quantities and steps employed being substantially the same as for production of a drier with any of the other metals (correction of course being had for different molecular weights).

The reaction is carried out in a closed kettle with suitable heating means, preferably a steam jacket, a reflux condenser communicating with the kettle through a trap from which water can be withdrawn while supernatant oil overflows back to the kettle. The kettle also contains a mechanical agitator.

The kettle is charged with 100 pounds (estimated for a mean molecular weight of 200) of coconut oil fatty acid, 400 to 500 pounds of naphtha and such a quantity of cobalt carbonate as will contain 14.1 pounds of cobalt, the theoretical equivalent of 95 to 97 pounds of the fatty acid.

The charge is stirred and heated so as to cause the naphtha to vaporize into the reflux condenser. Carbon dioxide liberated in the reaction escapes from the head of the condenser. Water liberated in the reaction is vaporized and condensed with the naphtha, but is removed by trapping out while the naphtha condensate returns to the charge. Reflux digestion is continued for as long as water continues to appear; then, reaction and dehydration being complete, the naphtha condensate is withdrawn until about 50 to 60 pounds of naphtha remains in the charge. The charge will now be a thick liquid if cooled to normal temperature and can be used very conveniently in that form. Alternatively, it may be made entirely free of naphtha and reduced to the solid, waxy

condition of maximum cobalt content by further evaporation preferably under vacuum.

The copper compound is made in the same way as above, using either normal or basic copper carbonate, in such quantity as to provide 15.3 pounds of copper, with the modifications that (1) due to the rapidity of the reaction the charge should be stirred for some time before heat is applied, and (2) due to the instability of the copper compound a more volatile grade of naphtha should be used and great care exercised to prevent local overheating, especially during the final reduction to solvent-free form.

The manganese compound is made the same way as the cobalt, using an amount of manganese carbonate to provide 13.2 pounds of manganese. The product is less stable than the cobalt compound but more so than the copper. Considerable care is required during the final reduction to solvent-free condition.

The lead and zinc compounds are made from the oxides in preference to the carbonates, using quantities to provide 49.6 pounds of lead or 15.7 pounds of zinc. The procedure is the same as for the cobalt compound except that, in the case of lead, the solvent content of the charge can be reduced to 40 or 50 pounds in the kettle and still yield a product sufficiently fluid to handle when cooled to normal temperature. The lead and zinc compounds are very stable.

The digestion and the procedure above outlined will ordinarily proceed for from one to four hours, the period varying according to conditions and even according to type of apparatus employed. Temperatures vary according to the "drying" metal being used; for instance, for the formation of copper fatty acid salts at an adequate rate, a temperature will be required above about 250° F., preferably around 350°, whereas manganese will require temperatures up to around 400° F. and cobalt up to around 450° or 500° F. These temperatures may be attained where naphtha is used as the solvent by employing a naphtha of greater or less volatility, or a lighter naphtha may be employed by operating under pressure. In addition to using oxides and carbonates of the drying metals mentioned, other compounds of these metals may be employed wherein the reaction products with the negative radicals will be eliminated in the digestion and distillation. For example the hydroxides, sulfides and salts of weaker volatile acids such as the acetates may be employed in some connections. In general a salt will be selected which is sufficiently stable and at the same time capable of insuring a sufficiently rapid rate of reaction. In case it is desired to avoid treatment in the presence of naphtha or similar solvent, an excess of fatty acid may be employed as a diluent and this excess eventually eliminated by distillation.

It is to be understood that the above disclosures are not to be considered as limiting of the generic invention disclosed, inasmuch as many variations may be made within the scope of the claims by those skilled in the art.

I claim:

1. A drier for paints and varnishes in the form of the mixed salt of the fatty acids of coconut oil in combination with a "drying" metal. 80

2. An oil soluble drier for paints, varnishes and the like comprising the fatty acid salts of coconut oil produced by combining coconut oil fatty acids with a metal of the class consisting of cobalt, copper, lead, manganese and zinc. 81

3. A drier produced by combining a drying metal of the class consisting of cobalt, copper, lead, manganese and zinc with the fatty acids of coconut oil, the drier readily forming a fine suspension by stirring in cold naphtha, this suspension being readily converted into a clear solution by heating to the boiling point of water without reprecipitation for several hours after cooling. 90

4. As an article of manufacture, a manganese-coconut oil acid product produced by combining manganese with coconut oil acids, the product having a waxy consistency and readily forming a fine suspension by stirring in cold naphtha. 95

5. An oil soluble drier produced by the combination of coconut oil fatty acids with a drying metal of the class including cobalt, copper, lead, manganese and zinc. 100

6. An article according to claim 5 which readily forms a fine suspension by stirring in cold naphtha, this suspension being converted into a clear solution by heating to the boiling point of water. 105

7. An oil soluble drier produced by combining a "drying" metal of the class consisting of cobalt, copper, lead, manganese and zinc with a mixture of capric, lauric and myristic acids, having a waxy consistency and being readily miscible in cold naphtha and readily soluble in naphtha at the boiling point of water. 110

8. An oil soluble drier in the form of a manganese-coconut compound resulting from the reaction of manganese with coconut oil acids, having a theoretical manganese content of at least 11%, having a waxy consistency and being readily soluble to a clear solution in naphtha at the boiling point of water. 120

9. A method for the production of oil soluble driers comprising commingling with coconut oil fatty acids a compound of a drying metal of the class consisting of cobalt, copper, lead, manganese and zinc, whose reaction products of its negative radical will be eliminated by distillation, and heating the mixture to a temperature and for a time to complete the conversion to salts of the fatty acids and to eliminate volatile products and constituents. 125

10. A method according to claim 9 wherein a relatively volatile solvent is added to the mixture and the reaction caused to take place in the presence of the solvent, and removing at least a part of the solvent by distillation. 130

11. A method according to claim 9 wherein the metallic compound is used in amount less than the theoretical amount required for conversion of the fatty acids. 140

ROBERT A. DUNHAM.